

Feb. 24, 1925.

1,527,959

C. F. SHERWOOD

PROCESS AND APPARATUS FOR MAKING SEATING MEMBERS FOR FLUID SEALS

Filed Oct. 25, 1922



FIG. 1.



FIG. 2.

INVENTOR

WITNESS:

R. P. R. Stichell.

Charles F. Sherwood  
BY  
Frank D. Busen  
ATTORNEY.

Patented Feb. 24, 1925.

1,527,959

# UNITED STATES PATENT OFFICE.

CHARLES FREDERIC SHERWOOD, OF SAN FRANCISCO, CALIFORNIA, ASSIGNOR OF  
ONE-HALF TO LYNDON E. ADAMS, OF PHILADELPHIA, PENNSYLVANIA.

## PROCESS AND APPARATUS FOR MAKING SEATING MEMBERS FOR FLUID SEALS.

Application filed October 25, 1922. Serial No. 596,734.

To all whom it may concern:

Be it known that I, CHARLES FREDERIC SHERWOOD, a citizen of the United States, residing at San Francisco, county of San Francisco, and State of California, have invented a new and useful Improvement in Processes and Apparatus for Making Seating Members for Fluid Seals, of which the following is a full, clear, and exact description, reference being had to the accompanying drawings, which form a part of this specification.

In the manufacture of metal covered gaskets, such, for example, as those used for sealing tube surfaces and specifically those interposed between the cap block and the removable head of a gasoline engine, it is customary to form a core or base by stamping or punching from a sheet of asbestos, fibre or other known substance and to form the cover by stamping or punching from a thin copper sheet; the metal cover being applied to the asbestos base and held thereon by crimping or other mechanical means. This method of manufacture is costly in the following respects: There is considerable waste of metal due to the punching out required to conform the metal sheet to the irregular form of the asbestos base and particularly to the large orifices contained therein. Much labor and some skill are required to fit and seal the metal sheet to the base and especially to crimp the edges of the sheet around the margin of the base and the edges of the orifices. Where the cover is made of copper, as it usually is, it is necessary to use electrolytically refined copper, which is quite expensive, while the waste copper is salable at but a small fraction of the cost, measured by weight, of the sheet metal.

It is known to provide a packing for pipe joints, piston rods, etc., having a body comprising an elastic substance as its main ingredient, rubbing graphite on the surface of the body to form an adhesive coating adapted to act as a cathode in an electrolytic bath, placing the same in such bath together with an anode, such as copper, and then connecting the anode and the graphite coated body with a source of electrical energy, thereby depositing on the graphite coated elastic body a coating of the material of the anode.

The object of my invention is to effect an

improvement in the known method of coating packing for pipe joints, piston rods, rubber valves for pumps, etc., which method is also applicable to asbestos gaskets for sealing tube surfaces and other seating, fluid-sealing and packing members that have been heretofore coated with metal or that have not heretofore been so coated but to which the application of a metal cover is desirable.

The object of my invention, more specifically stated, is to effect the execution of the foregoing process of electrolytic deposition of the copper or other desired metal covering in a more expeditious manner than heretofore, to manufacture a large number of the gaskets in a continuous manner, and to permit the use of a greater current density.

### In the drawings:

Fig. 1 is a face view of an uncoated asbestos gasket. Fig. 2 is a view of an apparatus for electrolytically coating in accordance with process.

Selecting a gasket of the type to which initial reference was made, which comprises a flat sheet of copper-covered asbestos having an oblong contour and provided with a series of rectangular perforations, the core or base *a* is first made as shown in Fig. 1 by stamping or punching the same from a sheet of asbestos, or by any other procedure, the method of forming the base having nothing to do with my invention. This base sheet is then dipped into a wax or gummed solution containing a large percentage of flake graphite or plumbago, or other suitable electro-conductive material.

A number of such graphitized asbestos gaskets are suspended from a conveyor *n* and travel successively through an electrolyte *o* contained in a vessel *p*, which is copper-lined and thus itself acts as the anode. The vessel and the conveyor are connected respectively with the opposite poles of an electric circuit.

By the foregoing method of manufacture, which is applicable to all seating, fluid-sealing and packing members, the rate of speed of the conveyor and the length of travel of the articles through the bath are so adjusted as to apply a coating of copper of the desired thickness by the time the article emerges from the bath. This method is also advantageous in that both the article to be metal-coated and the bath itself are subject-

ed to more or less agitation, thereby permitting the use of a greater current density.

Having now fully described my invention, what I claim and desire to protect by Letters Patent is:

1. The process of making a seating member for a fluid seal comprising forming a multiplicity of cores of a relatively electrically non-conductive material shaped in accordance with the desired shapes of the ultimate products, applying coatings of graphite thereto, and conveying the same successively through an electrolyte in contact with an anode concurrently with the passage of an electric current.

2. The process of making a seating member for a fluid seal comprising forming a multiplicity of cores of a relatively electrically non-conductive material shaped in accordance with the desired shapes of the ultimate products, dipping the cores into an adhesive solution containing graphite,

and conveying the cores successively through an electrolyte in contact with an anode concurrently with the passage of an electric current.

3. The process of making a seating member for a fluid seal comprising forming a multiplicity of cores of a relatively electrically non-conductive material shaped in accordance with the desired shapes of the ultimate products, applying coatings of graphite thereto, providing a vessel containing an electrolyte coated with the metal to be deposited on the cores, connecting the conveyor and the vessel with the opposite poles of an electric circuit, and passing the graphitized cores in a processional manner through the electrolyte concurrently with the passage of an electric current.

In testimony of which invention, I have hereunto set my hand, at New York, on this thirteenth day of October, 1922.

CHARLES FREDERIC SHERWOOD.